

## UNITED STATES PATENT OFFICE.

THEODORE MOTT, OF HOUSTON, TEXAS, ASSIGNOR TO B. F. GREENWOOD, OF HOUSTON, TEXAS.

## PAINT.

1,089,662.

No Drawing.

Specification of Letters Patent. Patented Mar. 10, 1914.

Application filed July 6, 1912. Serial No. 707,974.

To all whom it may concern:

Be it known that I, THEODORE MOTT, a citizen of the United States, residing at Houston, in the county of Harris and State 5 of Texas, have invented a new and useful Paint, of which the following is a specification.

This invention relates to paint compounds, its object being to provide a paint especially 10 designed for use in the treatment of wood so as to protect it from worms, to preserve it when under water, and to render it fire-proof.

A further object is to provide a paint 15 which will not crack, peel or run in hot weather.

The invention consists primarily in a combination of ingredients proportioned as follows:—Venetian red 10 lbs., salt 10 lbs., 20 brown mineral 10 lbs., sulfur 15 lbs., Cayenne pepper 2 lbs., rosin 15 lbs., water-gas tar 1 lb., gasolene or kerosene 1 pt.

In the preparation of the paint the ingredients above mentioned, with the exception 25 of the tar and the gasolene or kerosene, are thoroughly mixed. They are then placed with the tar and heated, the mixture being thoroughly stirred during the heating operation. The rosin, which is thoroughly 30 pulverized before being placed in the mixture, separates from the balance of the mixture during the first portion of this heating operation and floats on top of the mixture while it is being stirred and until the rosin 35 is completely melted whereupon further stirring of the mixture will result in the thorough commingling of the rosin with the other ingredients. While the paint is hot it is applied to the wood to be protected and,

when cool, forms a hard glazed surface 40 which renders the wood water and fire proof.

It has been found that the brown mineral constituting one of the ingredients of the paint, and which is a rocky formation containing an excess of iron oxid, is advantageous in that it gives the composition the quality of being impervious and unchangeable in all kinds of weather, especially in hot weather, thus preventing the paint from softening and giving it a high gloss. The 50 Venetian red serves to blend the colors and produces an attractive paint. The salt (NaCl) and the tar form a mixture which will not easily ignite and which therefore produces a fire proof coating. The pepper 55 permeates the wood and thus serves to protect it from the ravages of worms and other wood pests.

While the paint is intended primarily for use on wood, it has been found to be a useful 60 protection for metal inasmuch as it protects it from rust and gives it an attractive appearance.

What is claimed is:—

A paint for rendering wood fire, water 65 and worm proof, consisting of Venetian red ten pounds, salt ten pounds, brown mineral ten pounds, sulfur fifteen pounds, Cayenne pepper two pounds, rosin fifteen pounds, water-gas tar one pound, and gasolene one 70 pint, substantially as described.

In testimony that I claim the foregoing as my own, I have hereto affixed my signature in the presence of two witnesses.

THEODORE MOTT.

Witnesses:

C. H. ELY KUNOLL,  
A. T. SMITH.

Copies of this patent may be obtained for five cents each, by addressing the "Commissioner of Patents.  
Washington, D. C."

565.2

X140.4